

May 26, 1931.

W. L. WEDGER ET AL

1,807,456

FIRE EXTINGUISHING COMPOSITION

Filed March 24, 1930



Inventors.

W. L. Wedger,

J. W. Edmonds.

By

Pattison, Wright & Pattison  
Attorneys

## UNITED STATES PATENT OFFICE

WALTER LIBBY WEDGER, OF BELMONT, AND JOHN WILEY EDMANDS, OF NEWTON HIGHLANDS, MASSACHUSETTS, ASSIGNEES, BY MESNE ASSIGNMENTS, TO CENTRAL RAILWAY SIGNAL COMPANY, INC., A CORPORATION OF MASSACHUSETTS

## FIRE EXTINGUISHING COMPOSITION

Application filed March 24, 1930. Serial No. 438,507.

This invention relates to improvements in a chimney fire extinguisher and compound therefor and the primary object of this improvement is to combine a fire extinguishing agent with a heat producing agent.

5 A further object of the invention is to combine a fire extinguishing agent and a heat producing agent in a suitable container.

Another object of the present invention is 10 to produce a fire extinguisher container or tube that contains a combined fire extinguishing agent and a fire or heat producing agent which releases the fire extinguishing gases of the composition while at the same time 15 maintaining the necessary heat independent of a fire separate from the said container such for instance as a fireplace, a furnace fire or even a fire in a chimney.

Another object of the invention is to combine 20 a fire extinguishing agent and a fire producing agent both of them contained within a tubular container that itself contains means for igniting the contents of said tubular container whereby the said ignited tubular container and the composition contained can be 25 lighted independently of any other means, the said lighting means igniting the fire producing element of the composition thus producing the heat necessary for releasing the 30 fire extinguishing gases of the composition, the same being capable of use either in a fireplace or the communicating chimney or a furnace or the chimney thereof by disconnecting (or not) the pipe of the chimney 35 connected therewith.

A further object of the invention is to 40 combine a heat or fire producing agent that at the same time produces oxygen for maintaining the fire and combining it with an agent which when heated by the heat of said fire producing agent, releases gases from the fire extinguishing agent which smothers the fire in the chimney which is to be extinguished, whereby a fire department or other 45 person always has ready for instant use means that contains all that is essential to extinguish a chimney fire irrespective of the heat or fire of the chimney, fireplace, furnace or range.

50 So far as we are aware, chimney fire ex-

tinguishes heretofore used necessitated a fire independent of the said extinguisher for producing the heat necessary for releasing the fire extinguishing gases, so that the usual well known efforts to extinguish a fire by putting 55 out the fire in the fireplace, chimney, furnace or range are all very different from the immediate use as set forth of the present invention for extinguishing a fire in the chimney above, which does not require getting to the 60 top of the chimney with the attendant dangers, such as delay and accident.

Other objects and purposes of the present improvement will appear from the following 65 description.

In the drawings:

Figure 1 is a perspective view of a chimney fire extinguisher which embodies the present improvement.

Fig. 2 is a vertical central sectional view 70 of that end of the container that holds the improved composition.

Figure 3 is a slight modification of Figures 1 and 2.

In carrying out our present improvement 75 we provide an elongated tubular container 1 that has in one end a suitable wooden handle 2, the said handle being attached to the tube in any desired manner. The handle however may be omitted without affecting the 80 broad idea of the present invention. The said tubular member 1 is made of a suitable length for burning approximately four or five minutes, which from experience has proven to be ample for completely extinguishing the fire in the said chimney. The 85 opposite end 3 of this paper tube is turned inward as shown and is provided with a suitable opening 4, the purpose of which will be presently specifically explained. This end 90 3 of the tube is enclosed by a paper cap 5 that preferably has in one end a wooden plug 6 that closes its upper end.

Surrounding the cap 5 is a paper bonnet 95 or enclosure 7 and between the cap and the bonnet is a fibre strip 9 that extends throughout the length of the cap 5 and its lower end 9' extending below the lower end 10 of the bonnet. This lower end 10 of the bonnet is pasted to the tube 1. Located on 100

the outer end of the plug 6 is a friction lighting composition 11.

Located in the opening 4 is a complementary friction composition 12 that extends 5 beyond the end 3 and has its inner portion communicating with a suitable burning composition 13.

This last described construction is the well known construction used in railway 10 signal fuses.

When the chimney fire extinguisher is to be used the strip 9 is pulled upward and the end 15 broken away for the purpose of exposing the said complementary friction 15 igniting composition 11. The cap 5 is then twisted so as to break substantially at the point 14. The cap being removed the igniting composition 12 of the tube 1 is exposed and then by friction between the compositions 11 and 12 as with an ordinary safety match the fire extinguisher is ignited and the same is ready to be instantly used in the manner hereinafter set forth.

The combined fire extinguisher and heat 25 producing composition 16 consists of the following ingredients which are preferably, though not necessarily compounded in the following proportions:

|                          | Per cent |
|--------------------------|----------|
| 30 Potassium perchlorate | 15.02    |
| Sulphur                  | 19.12    |
| Zinc dust                | 49.14    |
| Ammonium chloride        | 5.46     |
| Magnesium carbonate      | 2.74     |
| 35 Potassium bichromate  | 1.70     |
| Wood pulp and paraffine  | 6.82     |

The function of these ingredients is as follows:

The potassium perchlorate is used as a 40 powerful oxidizing agent, which is very insensitive to friction or concussion, much more so than potassium chlorate. When this oxidizing agent is combined with sulphur, as it is here, it generates temperatures in a 45 burning composition approximately from 1900 to 2100° Fahr. thus furnishing heat necessary for vaporization of the other chemicals into their respective fire extinguishing gases. When the potassium perchlorate is being 50 burned it sets free a mixture of hydrogen chloride and chlorine gases in which fire cannot burn.

The sulphur is used in the fire extinguishing composition here disclosed both as a 55 reducing agent for the oxygen contained in the potassium perchlorate and, in large excess of what would be needed as a reducing agent, for the purpose of generating sulphur dioxide gas, which derives its two atoms of 60 oxygen from the oxygen of the perchlorate and from the air in the chimney. Large volumes of sulphur dioxide in which fire cannot burn are thus set free in the chimney.

Zinc dust is used in large percentage in 65 this chimney fire extinguishing formula. By

virtue of the heat generated by the combustion of potassium perchlorate and sulphur, the zinc dust is fused to zinc oxide which is drawn up the chimney by the draft and is deposited as a white or slightly gray, incombustible powder upon the inner surfaces of the chimney flue thereby retarding combustion in the burning soot and depriving it of the necessary oxygen to burn. The specific gravity of zinc oxide is 5.78 to water 1. This 75 heavy salt attaching itself to the accumulation of soot in the chimney we find pulls the soot down by its weight and is frequently used to clean chimney flues.

Ammonium chloride when subjected to 80 heat sublimes in part and under extreme heat is dissociated into its respective gases ammonia and chlorine or hydrogen chloride. These gases with the sublimed ammonium chloride are drawn up the chimney by the 85 draft, the former acting as an extinguishing agent by depriving the burning soot of the oxygen necessary to maintain fire, and the latter depositing itself upon the inner surfaces of the chimney flue acts as a fire retardant in addition to that deposited by the zinc oxide, whereby the whole exerts a cooling effect on the walls of the flue.

Magnesium carbonate is used in this chimney fusee composition both as an anti-acid to 95 correct any acid generation in the sulphur upon long keeping, and also when subjected to heat sets forth carbon dioxide gas which is drawn up the chimney by the draft and exerts its well known extinguishing influence.

Potassium bichromate is an oxidizer and it is used in small percentage in this composition as it has been found to react with the zinc dust, thereby producing a smoother burning mixture.

Wood pulp and paraffin is composed of wood treated with hot paraffin which on combustion generates carbon dioxide gas. This mixture together with a small amount 110 of paraffin oil is used to lay dust in handling the whole compound and also to make it pack firmer in the tubes or containers.

Ammonium chloride might possibly be omitted and obtain a useful extinguishing 115 fusee, but it would take longer to extinguish the fire in the burning soot and since a fire burning in a chimney for a long time would heat the bricks thereof to red-heat, the ammonium chloride is an important factor to 120 prevent the bricks becoming so hot as to communicate fire to the adjacent woodwork. Such an omission would be at the sacrifice of part of the extinguishing gases produced by it and the composition would lose the 125 rapid cooling effect since ammonium salts are endothermic.

The magnesium carbonate could be omitted and still have a usable extinguishing 130 fusee, but here again we would be losing part

of the extinguishing gases, viz. carbon dioxide. This chemical also has another function, that is to say, regardless of the sulphur used even if at the time of compounding it is 5 neither acid nor alkaline, sulphur gradually generates free sulphuric acid which reacts with the potassium perchlorate robbing it of part of its oxidizing content and thereby diminishing combustion and ultimate heat 10 for the vaporization of the chemicals into gases, but the presence of the magnesium carbonate instantly neutralizes all free acid generation, leaving the perchlorate to exercise its normal function. Magnesium carbonate 15 therefore contributes materially to the long keeping qualities of the composition and furnishes a valuable extinguishing gas.

The wood pulp, paraffin and paraffin oil might be omitted, but they likewise burn to 20 produce carbon dioxide in large volumes and to act as a dust layer in compounding the composition and to make it more capable of being packed hard in the tube. It also to a large extent acts as an internal water-proofing agent should the device be subjected to extreme dampness.

The fusee does not require and is never intended to be used from the top of the chimney thus requiring firemen to climb over the 30 roofs which is especially difficult and dangerous in the winter time when chimney fires are so frequent. It is a well known fact that chimney fires constitute the major portion of fire loss during the cold season in many localities, and hence the importance of a 35 convenient means for quick extinguishment of chimney fires. When we consider that the greater number of chimney fires takes place in flues connected with open fireplaces and 40 are caused by burning waste paper or other combustible matter in too large quantities, and when we consider that chimney fires are frequently caused by accumulations of oil soot in flues connected with oil burning equipment, which does not present in a firebox or 45 fireplace a solid bed of live coals for converting the extinguishing compounds into the fire extinguishing gases, the many advantages of the present improvement can be 50 readily appreciated.

The invention herein set forth and claimed has been and is being successfully used by the fire departments in several of the cities 55 where it has been in all cases reported efficient for quickly extinguishing a chimney fire by the use of one of the extinguishers described and defined in this application.

Having thus described our invention what 60 we claim and desire to secure by Letters Patent is:

1. A fire extinguishing composition consisting of potassium perchlorate, sulphur, zinc dust, the parts combined to simultaneously maintain combustion and generating a

fire extinguishing gas, for the purpose set forth.

2. A fire extinguishing composition consisting of potassium perchlorate, sulphur, zinc dust and potassium bichromate, said ingredients combined and operating for the 70 purpose set forth.

3. A fire extinguishing composition consisting of potassium perchlorate, sulphur, zinc dust, ammonium chloride, magnesium 75 carbonate and potassium bichromate, the said ingredients combined for the purpose set forth.

4. A fire extinguishing composition consisting of perchlorate, sulphur, zinc dust, ammonium chloride, magnesium carbonate, potassium bichromate, wood pulp and paraffin, the parts combined for the purpose set forth.

5. A fire extinguishing composition consisting of potassium perchlorate, sulphur, zinc dust, ammonium chloride, magnesium carbonate, potassium bichromate, wood pulp and paraffine, the ingredients combined in about the proportions herein set forth.

6. A fire extinguishing composition consisting of potassium perchlorate 15.02%, sulphur, 19.12%, zinc dust 49.14%, ammonium chloride 5.46%, magnesium carbonate 2.74%, potassium bichromate 1.70%, and wood pulp 95 and paraffine 6.82%, combined for the purpose set forth.

In testimony whereof, we hereunto affix our signatures.

WALTER LIBBY WEDGER.  
JOHN WILEY EDMANDS.

100

105

110

115

120

125

130